

Aug. 11, 1936.

W. SCHNEIDER

2,050,588

MANUFACTURE OF ANTIHALATION OR FILTER LAYERS

Filed Jan. 15, 1932

Fig. 1



Fig. 2



Fig. 3



Inventor  
Wilhelm Schneider  
By Attorneys  
Peter Pearce & Schaffler

## UNITED STATES PATENT OFFICE

2,050,588

MANUFACTURE OF ANTI-HALATION OR  
FILTER LAYERSWilhelm Schneider, Dessau in Anhalt, Germany,  
assignor to Agfa Anseco Corporation, Binghamton, N. Y., a corporation of New YorkApplication January 15, 1932, Serial No. 586,966  
In Germany January 21, 1931

14 Claims. (Cl. 95—8)

My present invention relates to anti-halation or filter layers for photographic materials.

One of its objects is to provide a method for producing anti-halation layers containing in uniform distribution an azo-dye which is insoluble in water. Another object is photographic materials provided with these anti-halation layers. Further objects will be seen from the detailed specification following hereafter. Reference is made to the accompanying drawing in which Figs. 1 to 3 show films or plates in accordance with the present invention in cross-section. In these figures 1 is the support, 2 is the emulsion layer. In Fig. 1 the film is provided with a filter layer 3 and in Figs. 2 and 3 the film is provided with an anti-halation layer 4.

I have found that anti-halation layers which do not bleed out in aqueous solutions and in the usual photographic baths and which can be decolorized in a simple manner may be obtained by developing the dye in a solution of a binding agent from its components and producing the layer from this mass. As water insoluble azo dyes which enter into consideration comprising mono- and poly-azo-dyes, I enumerate the coupling products of, for instance, aniline, naphthylamine, benzidine, diaminocbazole, diaminodiphenylene oxide, and the substitution products thereof with the coupling components, for instance, phenols, naphthols and the substitution products thereof. As binding agents for my new anti-halation layer suitable colloids may be used, for instance, gelatine, the calcium salt of poly-glycuronic acid and caseine.

The solution of the binding agent is mixed with the coupling component while adding the required amount of alkali, for instance, sodium hydroxide or sodium carbonate, whereupon the diazo-component is added to this mixture while stirring. After having become solid the mass is reduced to small pieces, for instance, cut in strips, and washed until its reaction has become neutral. From the resulting product the casting solution is made in known manner. In this manner very high concentrations of the dye in the layer may be obtained.

The layers may be provided between the support and the light sensitive emulsion layer or above the emulsion layer, or they may be provided on the rear side of the support. The layers can be easily decolorized by destroying the dye with the aid of an oxidizing reversal bath known from the usual photographic reversal methods, for instance, a solution of potassium permanganate and sulfuric acid. When working accord-

ing to the reversal method a special bath for removing the coloration of the anti-halation layer can, therefore, be dispensed with. When using the usual negative developing process, after the developing and fixing operation the negative may be treated with an oxidizing bath, for instance, an aqueous solution of 2 grams of potassium permanganate and 10 cc. of sulfuric acid per liter, which bath contains a halide, whereupon the produced silver-halide picture is transformed into a stable silver picture by means of a second exposure and a subsequent reduction by means of a developer or a suitable agent, for instance hydrosulfite.

The following examples illustrate the invention:

*Example 1.*—A solution of 70 parts by weight of gelatine in 800 parts by weight of water is cooled to 25° C. and mixed with 100 parts by weight of a  $\frac{1}{10}$  molal solution of sodium beta-naphtholate and 3 parts by weight of anhydrous sodium carbonate. Then 100 parts by weight of  $\frac{1}{10}$  molal diazo solution of alphanaphthylamine are slowly introduced, while stirring. The solution immediately becomes intensely red. It is caused to solidify, cut into small pieces and washed with water. After it has been molten, it is utilized in the usual manner for bottom coatings for the emulsion layer or for coating the surface of the emulsion layer or, if required, also the back layer of the support.

*Example 2.*—A violet colouration is obtained by using in Example 1 instead of the diazo solution of alphanaphthylamine 100 parts by weight of a  $\frac{1}{20}$  molal diazo solution of dianisidine.

*Example 3.*—A solution of 50 to 100 parts by weight of gelatine in 800 parts by weight of water is mixed with 100 parts by weight of  $\frac{1}{10}$  molal solution of sodium  $\beta$ -naphtholate and 3 parts by weight of sodium carbonate. To this mixture kept at about 25° C. there are added 100 parts by weight of a  $\frac{1}{20}$  molal diazo solution of benzidine. The solution becomes immediately dark red. The further working up of the mass is as described in Example 1.

*Example 4.*—When replacing in Example 3 the  $\frac{1}{10}$  molal solution of sodium  $\beta$ -naphtholate by a  $\frac{1}{10}$  molal solution of 1,7-aminophenol and the  $\frac{1}{20}$  diazo solution of benzidine by a  $\frac{1}{20}$  diazo solution of dianisidine a greenish blue mass is obtained which yields layer having a nearly black appearance when being about 5 to 6  $\mu$  thick.

*Example 5.*—A fuchsine-red solution of gelatine is obtainable by using equal parts of a  $\frac{1}{10}$

molal solution of sodium  $\beta$ -naphtholate and of a  $1/20$  molal diazo solution of toluidine.

Example 6.—A blue solution of gelatine with a cast to red is obtainable by using equal parts of 5 a  $1/6$  molal solution of sodium  $\beta$ -naphtholate and a  $1/20$  molal diazo solution of dianisidine.

My invention is not limited to the foregoing examples nor to the specific details given therein and I contemplate as included within my invention 10 all such modifications and equivalents as fall within the scope of the appended claims.

The term anti-halation layer as used in the specification and the claims is to include anti-halation layers and filter layers.

15 What I claim is:

1. A method of producing anti-halation layers which comprises mixing a solution of a binding agent with a coupling component of an azo dye of the group consisting of mono- and polyazo dyes

20 and alkali, adding to this mixture a diazo component, while stirring, reducing the mass after it has become solid to small pieces, washing the pieces until their reaction has become neutral 10 and preparing the anti-halation layers from this product.

25 2. A method of producing anti-halation layers which comprises mixing a solution of 70 parts by weight of gelatine in 800 parts by weight of water with 100 parts by weight of a  $1/6$  molal solution of 30 1.7-aminonaphthol, and 3 parts by weight of anhydrous sodium carbonate cooling the mixture to about 25° C., adding slowly while stirring 100 parts by weight of a  $1/20$  molal diazo solution of dianisidine, reducing the mass after it has become 35 solid to small pieces, washing the pieces until their reaction has become neutral, and preparing the layers from this product.

3. A method of producing anti-halation layers which comprises mixing a solution of 70 parts 40 by weight of gelatine in 800 parts by weight of water with 100 parts by weight of a  $1/6$  molal solution of sodium  $\beta$ -naphtholate, and 3 parts by weight of anhydrous sodium carbonate, cooling the mixture to about 25° C., adding slowly while 45 stirring 100 parts by weight of a  $1/6$  molal diazo solution of  $\alpha$ -naphthylamin, reducing the mass after it has become solid to small pieces, washing the pieces until their reaction has become neutral, and preparing the layers from this product.

50 4. A method of producing anti-halation layers which comprises mixing a solution of 70 parts by weight of gelatine in 800 parts by weight of water with 100 parts by weight of a  $1/6$  molal solution of sodium  $\beta$ -naphtholate, and 3 parts by weight of 55 anhydrous sodium carbonate cooling the mixture to about 25° C., adding slowly while stirring 100 parts by weight of a  $1/20$  molal diazo solution of benzidine, reducing the mass after it has become solid to small pieces, washing the pieces until

their reaction has become neutral, and preparing the layers from this product.

5 5. A method of producing anti-halation layers which comprises mixing a solution of gelatine with a coupling component of an azo dye of the group consisting of mono- and polyazo dyes and alkali, adding to this mixture a diazo component, while stirring, reducing the mass after it has become solid to small pieces, washing the pieces until their reaction has become neutral 10 and preparing the anti-halation layers from this product.

15 6. A photographic material which comprises a support, a light sensitive silver-halide emulsion and an anti-halation layer comprising a binding agent and an azo dye, said azo dye being insoluble in water.

20 7. A photographic material which comprises a support, a light sensitive silver-halide emulsion and an anti-halation layer comprising a binding agent and an azo dye, said azo dye being insoluble in water, but soluble in the oxidizing reversal baths.

25 8. A photographic material which comprises a support, a light sensitive silver-halide emulsion, and an anti-halation layer comprising a binding agent and an azo dye, said azo dye being insoluble in water, but soluble in a solution of potassium permanganate and sulfuric acid.

30 9. A photographic material which comprises a support, a light-sensitive silver halide emulsion and an anti-halation layer containing the azo dye from 1.7-amino-naphthol and di-anisidine.

35 10. A photographic material which comprises a support, a light-sensitive silver halide emulsion and an anti-halation layer containing the azo dye from sodium  $\beta$ -naphtholate and  $\alpha$ -naphthylamine.

40 11. A photographic material which comprises a support, a light-sensitive silver halide emulsion and an anti-halation layer containing the azo dye from sodium  $\beta$ -naphtholate and benzidine.

45 12. A photographic material which comprises a support, a light sensitive silver halide emulsion and an anti-halation layer comprising gelatin containing an azo dye insoluble in water.

50 13. A photographic material which comprises a support, a light sensitive silver halide emulsion and an anti-halation layer comprising gelatin containing an azo dye insoluble in water but soluble in oxidizing reversal baths.

55 14. A photographic material which comprises a support, a light sensitive silver halide emulsion and an anti-halation layer comprising gelatin containing an azo dye insoluble in water but soluble in a solution of potassium permanganate and sulfuric acid.

WILHELM SCHNEIDER.